



US005848579A

# United States Patent [19]

Adachi et al.

[11] Patent Number: 5,848,579

[45] Date of Patent: Dec. 15, 1998

[54] CYLINDER HEAD FOR ENGINE

[75] Inventors: **Shuhei Adachi; Junichi Inami**, both of Iwata, Japan[73] Assignee: **Yamaha Hatsudoki Kabushiki Kaisha**, Iwata, Japan

[21] Appl. No.: 638,981

[22] Filed: Apr. 25, 1996

## [30] Foreign Application Priority Data

Apr. 26, 1995 [JP] Japan 7-102004

[51] Int. Cl.<sup>6</sup> F01L 3/22

[52] U.S. Cl. 123/188.8

[58] Field of Search 123/193.5, 193.3, 123/188.8, 188.9

## [56] References Cited

## U.S. PATENT DOCUMENTS

4,723,518 2/1988 Kawasaki et al. 123/188.8

|           |         |                 |           |
|-----------|---------|-----------------|-----------|
| 4,734,969 | 4/1988  | Kuroishi et al. | 123/188.8 |
| 4,791,259 | 12/1988 | Pfaffmann       | 128/188.8 |
| 4,934,351 | 6/1990  | Shepley         | 123/188.8 |
| 5,020,490 | 6/1991  | Seko            | 123/188.8 |
| 5,564,187 | 10/1996 | Sihon           | 123/188.8 |
| 5,586,530 | 12/1996 | Adachi et al.   | 123/188.8 |
| 5,632,240 | 5/1997  | Sihon           | 123/188.9 |
| 5,687,685 | 11/1997 | Amano et al.    | 123/188.8 |

Primary Examiner—Marguerite McMahon  
Attorney, Agent, or Firm—Knobbe, Martens, Olson & Bear  
LLP

## [57] ABSTRACT

A cylinder head assembly for an internal combustion engine having a bonded valve seat. The cylinder head material is chosen as an aluminum alloy that has certain physical and electrical characteristics so as to improve the bonding strength between the cylinder head and the insert which forms in substantial part the valve seat.

20 Claims, 11 Drawing Sheets





**Figure 1**  
*Prior Art*



**Figure 2**  
*Prior Art*



**Figure 3**



**Figure 7**



**Figure 4**



**Figure 5**



**Figure 6**



**Figure 8**



**Figure 9**



**Figure 10**



**Figure 11**



**Figure 17**



**Figure 12**



**Figure 13**



**Figure 14**



**Figure 15**



**Figure 16**



**Figure 18**



**Figure 19**



**Figure 20**

## CYLINDER HEAD FOR ENGINE

## BACKGROUND OF THE INVENTION

This invention relates to a valve seat arrangement for a reciprocating machine and more particularly to an improved cylinder head having bonded valve seats for an internal combustion engine.

In internal combustion engines, it frequently is the practice to employ aluminum or aluminum alloys as the material for a number of the major engine castings such as the cylinder heads. When the cylinder heads are formed from aluminum or aluminum alloys, however, certain components of the cylinder head are formed from a dissimilar material so as to improve performance. For example, the valve seats of the cylinder head are normally formed from a harder, less heat conductive material such as iron or ferrous iron alloys. By utilizing such harder materials, the valve seat life can be extended. However, the attachment of the dissimilar valve seat insert into the cylinder head presents a number of problems.

Conventionally, it has been the practice to form the cylinder head passages with recesses adjacent the seating area into which the insert rings which form the valve seat are press fit. The use of press fitting has a number of disadvantages. These disadvantages may be understood by reference to FIG. 1 which shows a conventional pressed in type of valve seat.

The cylinder head material 21 is formed with a counterbore 22 at the cylinder head recess side of the flow passage 23. The flow passage 23 may be either an intake passage or an exhaust passage. The insert ring is indicated by the reference numeral 24 and may be formed from any suitable material, such as a Sintered ferrous material. Such materials have the advantage of having high wear capabilities. After the insert 24 has been pressed into place, its surface is machined as at 25 so as to form the actual valve seating surface.

As may be seen, this technique requires relatively large valve seat inserts in order to withstand the pressing pressures. In addition, the press fit must be such that the insert ring will not fall out when the engine is running. As a result, there are quite high stresses exerted both on the cylinder head and on the insert ring. The stresses can result in loads which may eventually cause cracks in the cylinder head.

These types of construction also limit the maximum size and spacing of the valve seats in order to ensure adequate cylinder head material between adjacent valve seats to reduce the likelihood of cracking. In addition, the large seats compromise the configuration of the intake passages, particularly at the critical valve seating area. Finally, these constructions result in somewhat poor heat transfer from the valve to the cylinder head due to the poor thermal conductivity of the valve seat material and the poor contact area between the insert 24 and the cylinder head 21.

In addition, the interface between the insert ring and the cylinder head frequently leaves voids or air gaps which further reduce the heat transfer and thus cause the valves to run at a higher temperature. This higher temperature operation of the valves requires the valves to be made heavier and stronger and thus reduce the performance of the engine and increase its size and costs.

Many of these problems become worse as the engine reaches operating or higher temperatures. Because of the higher coefficient of expansion of the cylinder head material, the press fit force diminishes and the contact area for heat transfer also decreases.

It has been proposed, therefore, to utilize a technology wherein the insert ring is laser clad into the cylinder head. Such a cylinder head assembly is shown in FIG. 2. In this technique, a somewhat smaller insert ring 26 is laser clad into the cylinder head material 21. This results in a bonding interface 27 that is formed between melt reaction layers 28 and 29 of the cylinder head material 21 and insert ring material 26. These actually form alloys.

Such laser cladding generally ensures against the likelihood of stresses which may cause cracking. Nevertheless, the laser cladding technique itself requires rather large inserts and thus a number of the disadvantages with pressed in inserts also are found with welded inserts. Furthermore, the heat transfer problems are also prevalent and in some instances can become worsened.

With a laser cladding technique, there is actually formed a metallurgical alloy between the material of the insert ring and the cylinder head. Because of the fusion process, air pockets or voids may occur in the areas 28 and 29 and heat transfer is reduced. In addition, the alloy at the interface between the insert ring and the cylinder head also has poor thermal conductivity and thus a number of the problems present with pressed in inserts are also present with laser clad inserts.

It has been proposed, therefore, to employ a technique wherein the insert ring is metallurgically bonded but not alloyed to the cylinder head material. This is accomplished by pressing the insert into place and passing an electrical current through the insert which is sufficient to cause the cylinder head material to plastically deform upon insertion of the insert ring. The plastically deformed phase of the cylinder head material forms a metallurgical bond at the interface with the insert ring without any significant resulting alloying of the cylinder head material to that of the insert ring. Such an arrangement is disclosed in our co-pending application entitled, "Valve Seat Bonded Cylinder Head and Method for Producing Same," application Ser. No. 08/483, 246, filed Jun. 7, 1995 and assigned to the assignee hereof. In addition, certain of these techniques are also described in our co-pending application entitled "VALVE SEAT," application Ser. No. 08/278,026, filed Jul. 20, 1994, in the names of Shuhei Adachi & Junichi Inami and also assigned to the Assignee hereof.

These techniques have a number of advantages over the conventional structures. First, they permit the use of much smaller insert rings since the pressing pressure is reduced and thus the shape of the intake passage, particularly the shape of the cylinder head passages, particularly in the critical area of the valve seats are not compromised. In addition, the bond strength is considerably higher than more conventional methods. Furthermore, this technique, because of the improved way in which the adhesion is formed, permits the use of much smaller insert rings and thus permits the valve seat openings to be positioned closer to each other without the likelihood of causing defects in the cylinder head which may manifest themselves during the engine running and life.

It has been found that the bond strength is dependent to a large extent upon the materials which are chosen, particularly for the cylinder head. Although this technique generally provides a stronger bond strength and requires greater separation forces to remove the insert than more conventional techniques, still further improvements can be obtained.

It is, therefore, a principal object of this invention to provide an improved bonded valve seat arrangement for a cylinder head.

It is a further object of this invention to provide a cylinder head incorporating a bonded valve seat wherein the cylinder head and valve seat insert materials are chosen so as to improve the bonding strength.

#### SUMMARY OF THE INVENTION

A first feature of this invention is adapted to be embodied in a cylinder head for an internal combustion engine comprised of a main cylinder head body formed from a first material. The main cylinder head body is formed with a surface adapted to be facing relationship to a cylinder block for closing a cylinder bore formed therein. A recess is formed in the main cylinder head body surrounded by the surface. A flow passage extends through the cylinder head body between the recess and an external surface of the main cylinder head body. A valve seat is formed at the recess end of the flow passage by an insert formed from a second material different from the first material and metallurgically bonded thereto. The first material comprises an aluminum alloy having a solidus temperature greater than 530° C.

A further feature of this invention is also adapted to be embodied in a cylinder head for an internal combustion engine comprised of a main cylinder head body formed from a first material. The main cylinder head body is formed with a surface adapted to be facing relationship to a cylinder block for closing a cylinder bore formed therein. A recess is formed in the main cylinder head body surrounded by the surface. A flow passage extends through the cylinder head body between the recess and an external surface of the main cylinder head body. A valve seat is formed at the recess end of the flow passage by an insert formed from a second material different from the first material and metallurgically bonded thereto. The first material comprises an aluminum alloy having a 0.2% yield strength at 400° C. less than about 35 M4Pa.

Another feature of this invention is also adapted to be embodied in a cylinder head for an internal combustion engine comprised of a main cylinder head body formed from a first material. The main cylinder head body is formed with a surface adapted to be facing relationship to a cylinder block for closing a cylinder bore formed therein. A recess is formed in the main cylinder head body surrounded by the surface. A flow passage extends through the cylinder head body between the recess and an external surface of the main cylinder head body. A valve seat is formed at the recess end of the flow passage by an insert formed from a second material different from the first material and metallurgically bonded thereto. The first material comprises an aluminum alloy having heat conductivity of greater than about 150° C. W/m.

Still another feature of this invention is adapted to be embodied in a cylinder head for an internal combustion engine comprised of a main cylinder head body formed from a first material. The main cylinder head body is formed with a surface adapted to be facing relationship to a cylinder block for closing a cylinder bore formed therein. A recess is formed in the main cylinder head body surrounded by the surface. A flow passage extends through the cylinder head body between the recess and an external surface of the main cylinder head body. A valve seat is formed at the recess end of the flow passage by an insert formed from a second material different from the first material and metallurgically bonded thereto. The first material comprises an aluminum alloy having an electrical resistivity of less than  $8.5 \times 10^{-2} \mu\Omega$ .

Yet another feature of this invention is adapted to be embodied in a cylinder head for an internal combustion

engine comprised of a main cylinder head body formed from a first material. The main cylinder head body is formed with a surface adapted to be facing relationship to a cylinder block for closing a cylinder bore formed therein. A recess is formed in the main cylinder head body surrounded by the surface. A flow passage extends through the cylinder head body between the recess and an external surface of the main cylinder head body. A valve seat is formed at the recess end of the flow passage by an insert formed from a second material different from the first material and metallurgically bonded thereto. The first material comprises an aluminum alloy comprised of aluminum, silicon and magnesium.

#### BRIEF DESCRIPTION OF THE DRAWINGS

FIG. 1 is an enlarged cross-sectional view taken through a conventional prior art-type pressed in valve seat.

FIG. 2 is an enlarged cross-section view, in part similar to FIG. 1, and shows a conventional laser clad type valve seat.

FIG. 3 is a partial cross-sectional view taken through a cylinder head having valve seats formed and constructed in accordance with the invention.

FIG. 4 is a front elevational view of an apparatus for practicing the invention for making bonded valve seats.

FIG. 5 is a side elevational view of the apparatus.

FIG. 6 is an enlarged cross-sectional view showing the apparatus in position for forming the bonded valve seat.

FIGS. 7-11 are step-by-step cross-sectional views showing the steps in pressing in and bonding a valve seat insert in accordance with the invention with FIG. 7 showing the initial step and FIG. 11 showing the final machined valve seat.

FIG. 12 is a graphical view showing pressing force and electric current flow in accordance with a preferred method of practicing the invention to achieve a bonded valve seat.

FIG. 13 is a graphical view showing the influence of electrical resistivity of the cylinder head material on the strength of the resulting bond, both as initially installed as shown in the open characterized views and after being held at 300° C. for 24 hours in the shaded line views.

FIG. 14 is a graphical view showing the effect of heat of conductivity of the cylinder head material on the separation strength, both after bonding and after the heating as mentioned in reference to FIG. 12.

FIG. 15 is a graphical view showing the effect of the solidus temperature on the separation load, both as installed and after heating.

FIG. 16 is a graphical view showing the effect of yield strength of the cylinder head material on separation load, both after bonding and after the heat test afore-referred to.

FIG. 17 is a top plan view showing a shield device that can be utilized with the pressing electrode to control the direction the eutectic alloy is removed from the bonded portion.

FIG. 18 is a cross-sectional view, in part similar to FIG. 7, and shows another configuration that may be employed for the insert and cylinder head.

FIG. 19 is an enlarged cross-sectional view, in part similar to FIGS. 7 and 18, and shows yet another configuration which may be employed for the insert and the cylinder head recess.

FIG. 20 is a cross-sectional view, in part similar to FIGS. 7, 18 and 19, and shows a still further configuration of insert that may be employed.

#### DETAILED DESCRIPTION OF THE PREFERRED EMBODIMENTS OF THE INVENTION

It should be noted that the actual mechanical way in which the bond is formed with the valve seat is as described in the

aforenoted co-pending applications, the disclosures of which are incorporated herein by reference. Even though these disclosures are incorporated herein by reference and the invention in this application deals primarily with the pressing method, a general description of the bonding process will also be included. However, where further information is required, reference may be had to the aforenoted co-pending applications.

Referring first to FIG. 3, a cylinder head for an internal combustion engine utilizing the invention is identified generally by the reference numeral 31. The cylinder head includes a base cylinder head casting 32 which is formed from an aluminum or aluminum alloy. Such materials are highly desirable for use in engine components and particularly cylinder heads because of their light weight and high thermal conductivity and specific, preferred materials will be disclosed later herein.

The cylinder head 32 is formed with combustion chamber recesses 33 which cooperate with the associated cylinder bore and piston (both of which are not shown) of the associated engine to form its combustion chambers. An intake charge is delivered to these combustion chambers through one or more intake passages 34 that are formed in the cylinder head material 32 and which terminate at valve seat 35 within the cylinder head recess 33. Poppet type intake valves 36 are supported within the cylinder head 32 by valve guides 37 for controlling the opening and closing of the valve seats 35 in a well known manner. The intake valves 36 may be operated by any known type of valve actuating mechanism.

One or more exhaust passages 38 extend from the cylinder head recesses 33 and specifically from valve seats 39 formed therein for the discharge of the combustion products from the combustion recesses 33 in a manner also well known in this art. Exhaust valves 41 are slidably supported in the cylinder head 32 by valve guides 42. These exhaust valves 41, like the intake valves 36 are operated by any known type of mechanism.

The invention, as should be readily apparent from the foregoing description, deals in the method in which the valve seats 35 and 39 are formed and the materials employed, particularly for the cylinder head casting. This apparatus is shown best in FIGS. 4-6 and will be discussed and described by reference to these figures.

The apparatus is indicated generally by the reference numeral 43 and may be considered to be similar to a pressure welding apparatus. However, and as will become apparent, the actual electrical current flow is not sufficient to cause any welding of the insert rings to the cylinder head material.

The apparatus 43 is comprised of a press base 44 that has a support element 45 on which a fixture 46 is mounted so as to accommodate a cylinder head 32. The fixture 46 is disposed so that the cylinder head 32 will be held at an angle. This angle is such that one of bores 47 or 48 (FIG. 3) that received the valve guides 37 or 42 will be in line with the pressing axis of the equipment.

Supported above the table or base 45 is a ram 49 which is driven by a hydraulic or pneumatic motor 51. The ram 49 carries a pressing electrode member, indicated generally by the reference numeral 52.

Affixed to the pressing electrode member 52 is an adjustable post 53 which cooperates with a proximity sensor or detector 54 such as a laser which is utilized to determine the degree of movement during the pressing of the inserts in place and the degree of movement of the ram 49 specifically. The output of this detector 54 indicates the depth at which the insert is pressed into the cylinder head, as will become apparent.

The base 44 carries a source of high energy electricity that is transmitted to the base plate 45 through a first conductor 55 and to the pressing member 52 through a second conductor 56. The conductors 55 and 56 will accommodate vertical movement and the conductor 56 is so configured in this embodiment. The pressing electrode 52 is preferably charged positively and the support base 45 is negatively charged.

The actual pressing apparatus and its association with the cylinder head will now be described by reference FIG. 6. As seen in this figure, a mandrel post, indicated generally by the reference numeral 57, is placed into the valve guide opening 47 of the cylinder head 32. The mandrel post 57 is formed from a central post part 58 that is formed from a suitable material, such as a metallic rod. However, in order to provide electrical insulation, for a reason which will become apparent, the rod 58 is provided with an insulating coating 59. Although the insulating coating 59 may be of any material, a ceramic material, such as alumina, is preferred. The alumina coating 59 is flame sprayed onto the rod base 58 and then is finished by polishing.

A stopper ring 60 is affixed to the mandrel 57 and contacts the inner surface of the cylinder head intake passage 34 around the valve guide opening 47 so as to limit how far the mandrel post 57 extends into the valve guide opening 47.

A further pressing member, indicated generally by the reference numeral 61, is provided with an opening 62 complementary in shape to the mandrel and is slid thereover. The pressing member 61 has an actual pressing surface that is formed by a hardened body 63 formed from an appropriate material and which either is magnetized or which carries a magnetic body 64 so as to attract and hold an insert ring 65 thereupon. The body surface 63 is formed with a tapered end 66 that is complementary to the shape of the insert ring 65, as will be described later by reference to FIG. 7. Because the pressing body 61 is engaged the electrode 52, electrical current will flow through the pressing body 61 and through the insert ring 65. As will become apparent later, when the insert ring 65 is engaged with the cylinder head 32, an electrical path will be formed through the cylinder head and base 45 to the conductor 55 to complete the electrical path. The insulated coating 59 on the mandrel 57 prevents short-circuiting around this area.

The construction of the insert ring 65, its shape and the shape of a cooperating recess 67 formed in the cylinder head at the mouth of the intake passage 34 will now be described by primary reference initially to FIG. 7. FIG. 7 is an enlarged cross-sectional view of one of the intake valve seats 35 and this description may be considered to be typical for that which may be utilized with the exhaust valves 41 to form the exhaust valve seats 39.

Basically, the valve seat 35 is formed by the insert ring, indicated by the reference numeral 65 and which has a metallurgical construction as will be described. This insert ring 65 is bonded to the cylinder head material 32 by a relatively thin metallurgical bonding layer that is formed in a manner which will be described. Adjacent this bonding layer, there is formed a portion of the material of the cylinder head 32 which has been plastically deformed. It should be noted that the alloy of the cylinder head 32 is of the same chemical composition and same physical structure, except for being slightly work hardened in the area adjacent the bonding layer, as in the remainder of the cylinder head material 32.

The insert ring 65, is formed from a Sintered ferrous alloy base 68 having a coating material filled within its intercices

and also on its external surface as desired, which coating is indicated at 69. This material is preferably formed from a good electrical conductor such as copper. Copper also has another useful function as a coating for a reason to be described.

The insert ring 65 in accordance with this embodiment is formed with a cylindrical inner surface 70 that is relatively short in axial length and which merges into a tapered conical surface 71 which extends for a substantially length. The surface 71, which is actually the pressing surface, as will be described, ends in an end surface 72.

First, conical outer surface section 73 extends at an acute angle to the axis of the cylindrical section 70 and merges at a rounded section 74 into an inclined lower end surface 75 which is formed at a greater angle than that of the conical surface 73. However, this angle is still an acute angle to a plane perpendicular to the axis of the cylindrical section 70.

The cylinder head material 32 is formed with a recess that is comprised of a first section 76 that is connected to a second section 77 that are joined by a horizontal surface that forms a projecting ledge 78 that contacts the rounded portion 74 of the insert ring 65 upon initial installation (FIG. 7). This tends to form a localized area that will begin the plastic deformation phase.

It has been noted that the copper coating serves the function of improving the electrical conductivity of the insert ring 65. Also, it has been noted that the copper performs additional functions. As should be apparent from the foregoing description, it is important that the bonding process not result in any alloying of the insert ring material and specifically that of the base 68 with the base material of the cylinder head 32.

The copper also serves the function of forming a eutectic alloy with the material of the cylinder head 32 which eutectic alloy has a lower melting point than either the melting point of the copper or that of the cylinder head material. As a result, the plastic deformation is accomplished with added ease and the metal can flow out during the pressing process as will be noted without large heat generation. In addition, the copper will react with any aluminum oxides that may be present on the surface of the recess 67 of the cylinder head 32 so as to extrude these oxides and provide a purer finish.

Preferably, the copper plating is done by electroplating and has a thickness in the range of 0.1–30  $\mu\text{m}$ . Also, the cylinder head material of the body 32 is preferably an aluminum alloy as set forth in Japanese Industrial Standard (JIS) AC4C. For reasons which will be noted later by reference to FIGS. 12 through 15 this material, which is an aluminum, silicon, magnesium based aluminum alloy, has higher bonding strength than the AC4B and AC2B aluminum, silicon, copper and aluminum, copper, silicon based aluminum alloys typically used for cylinder head castings.

Beginning now to describe the pressing operation by reference to FIGS. 7–11, FIG. 7 shows the conditions comparable to that in FIG. 6. The pressing force is then applied by actuating the hydraulic ram operating motor 51 so as to move the electrode 52 into contact with the pressing mandrel electrode 61. Prior to this the mandrel 61 may be rotated to ensure that the insert ring 65 is correctly seated.

A pressing force is then applied at a force indicated at the force P1 in FIG. 12. This force acts along the center axis of the seat and is maintained up until the time T1 wherein an electric current flow through the joint is initiated. When this occurs, there will be a high electrical resistance due to the

small contact area and a plastic deformation begins in the range indicated at A in FIG. 8 so as to displace the material of the cylinder head 32.

As the current is built up, the material will reach a temperature wherein the internal resistance is high enough to cause the copper coating layer 74 to diffuse into the cylinder head material in the area 78 or shown in the range A so as to form the eutectic alloy that results in the area indicated at A in FIG. 8 and which eventually causes displacement and a plastic deformation and the insert ring 65 will begin to become embedded in the material of the cylinder head 32.

The eutectic layer is displaced as indicated at B in FIG. 9 toward the area which will be removed from where the final valve seat will be formed. Said another way, this material will be later machined away.

The actual deformation of the insert into the cylinder head body, as measured by the sensor 54, begins at the point in time T2. At some time thereafter, the electric current will have reached its maximum amount at the first level at the point T3 and then the pressing pressure is increased from the pressure P1 to a new higher pressure P2 which is then held.

This plastic deformation then continues and after a certain deflection and at the time period T4, the electric current is reduced sharply toward zero as shown in FIG. 12. This is done to avoid overheating and to ensure that there will be no alloying of the insert ring material and that of the cylinder head material. There will, however be atomic diffusion of the materials in the area C.

The electric current is then built up higher to a new level equal to or slightly higher than that before and is held at this level until the point in time T5. This pressing is continued after this still at the pressure P2 during which time period the current flow is dropped back to zero at the time period T6 while pressing is continued. The final joint appears as shown in FIG. 10 and it will be seen that substantially all of the eutectic alloy has been pushed from the area between the insert base 68 and the base cylinder head material resulting in only the work hardened adjacent the joint and atomic bonding in the area C. In addition, the metallurgical bonding will be completed.

During this time and after the completed bonding, the apparatus measures the amount of actual embedding of the insert ring 65 into the cylinder head 32. There is an allowable range as indicated by the dimension D in FIG. 12 which range is about 0.5 millimeters to 2 millimeters and preferably in the range of 1 to 1½ millimeters. If the sinking level is not reached in this range, then it can be assumed that the joint is not satisfactory. This judgment may also be made during the actual pressing, bonding operation. If the deflection is not in the proper range, the process may be discontinued.

In addition, a judgment may be made whether the main current values and total energization time are in the allowable range. If this is also met, then certain cylinder head valve seats may be actually pull testing to assure accuracy and satisfaction of the entire lot of cylinder head formed.

The way this testing is done is that a tensile force is applied by putting an appropriate fixture under the projecting edge of the insert ring as shown in FIG. 10 and applying a pulling force. This way, the actual force necessary to separate the bonded joint can be measured. If the samples are within the predetermined range, then it can be assumed that all heads in the lot, which have also passed the other test, are satisfactory.

In addition to these tests, there can be a heat endurance test and/or heat shock test applied to the finished cylinder head. All of these things are done before the final machining.

The heat endurance test is performed on the cylinder head in the state shown in FIG. 10. The head is kept in a furnace at 300° C. and atmospheric pressure in the range of 24 to 200 hours. A further pulling test is then performed and the area inspected for separation or cracks. In a heat shock test, the finished cylinder head in the condition shown in FIG. 10 is heated to 300° C. in a furnace at that temperature and atmospheric conditions. The thus heated head is then immediately immersed in ice water at 0° C. This procedure is repeated ten times and then the cylinder head is checked for separation and cracks and the separation test aforesaid is performed.

Assuming that the tests indicate that the head lot is satisfactory, then the heads are finish machined by grinding or the like to the conditions shown in FIG. 11. Thus, it will be seen that all of the eutectic alloy phase B is removed and only the metallurgical bonding area C remains. The finished joint has no melt reaction layer or no actual alloying between the cylinder head material and that of the insert ring.

A visual inspection is also made after the bonding is completed. In this inspection it is checked to see that the eutectic alloy portion B (FIG. 10) extends around the entire insert without voids. If not the piece should be rejected as the bond may have voids.

As has been noted, the aluminum silicon magnesium-based aluminum alloy AC4C has been chosen because it has been found to provide a higher bonding strength than other aluminum alloys normally used for cylinder head castings. The reason for this will be described by particular reference to FIGS. 13-16 which show certain comparisons between this material and JIS AC4B, an aluminum silicon copper-based aluminum alloy, and AC2B, an aluminum copper silicon-based aluminum alloy. These are the materials that are more conventionally used for aluminum alloy cylinder head castings.

In FIGS. 13-16, the symbols  $\bigcirc\bullet$  represent the material AC4C before and after the heating test. The heating test, as previously noted, soaks the cylinder head at a temperature of 300° C. for 24 hours and then lets it be air cooled before testing.

The symbols  $\diamond\blacklozenge$  represent the material AC4B after the same conditions and the symbols  $\square\blacksquare$  represent the material AC2B.

As seen in FIG. 13, the electrical resistivity of the conventional materials is in the order of  $8.5 \times 10^{-2}$   $\mu\Omega\cdot M$  compared to the much lower value of about  $7.1 \times 10^{-2}$   $\mu\Omega\cdot M$  for this preferred AC4B material. Because of the lower resistivity of this material from the conventional materials, the current flow results in less generation of heat and there is less likelihood of localized melting and more even heat transfer across the joint during its formation.

FIG. 14 also shows how this heat conductivity, which for the chosen material is substantially higher than 120  $W/m\cdot C$  which are the higher heat conductivities for the conventional material. In fact, the heat conductivity for the AC4B is more in the range of 160  $W/m\cdot C$ . Again, the increased separation load is obvious.

FIG. 15 shows another characteristic of the cylinder head material which is found to produce better results and this is its substantially higher solidus temperature. As known, this is the temperature at which the material transforms from solid phase to liquid phase. The conventional materials have a solidus temperature of 520° C. and, hence, it is more likely that they will turn to a liquid and cause alloying. The preferred material has a solidus temperature of about 555° C. and, thus, results in a stronger joint.

A further characteristic which is found to produce better bonding is if the material has a lower 0.2% yield strength at 400° C. than the conventional materials. Again, this appears to result in more plastic flow than would be possible with the conventional materials as shown in FIG. 16. The yield strength is preferably substantially below 45 MPa and, preferably, in the range of 30-35 MPa.

FIG. 17 shows another embodiment of the invention and in this embodiment the electrode 52 of the pressing head is provided with a ferrous semi-circular shield 101 which functions to provide a magnetic flux in the magnetic field which directs the eutectic alloy that is removed from the bonded area. This can be done so as to ensure that more of the eutectic alloy is disposed in the area where the most machining will occur so as to minimize the amount of machining necessary. Also this is done to insure complete bonding around the joint.

In the foregoing description, a specific shape of insert and cylinder head recess has been depicted and described. The insert and recess may take different configurations as shown in FIGS. 18-20. FIG. 18 shows a configuration similar to that of the previous embodiment, but the cylinder head recess is merely formed with a simple taper. In addition, the insert is not rounded, but the bonding operating will begin at a small area as in the previously described embodiment.

FIG. 19 shows another embodiment using a different shape ring and that lends itself to what is called end pressing. However, the shape of the insert ring is again such that the initial deformation of the cylinder head will begin at the middle of its tapered area. In addition, an outer peripheral groove will assist in locating.

FIG. 20 shows a simplified form of shape of insert ring that adapts itself to the pressing method which can be utilized with all of the embodiments of FIGS. 1-14. Again, however, the arrangement is designed so as to ensure localized initial deformation. Also, each of these embodiments are designed so as to provide the desired length of bonding surface to provide the desired bonding strength. Also, although a specific cylinder head material and insert material have been disclosed, various other materials may also be practiced.

Thus, from the foregoing description it should be readily apparent that the described cylinder head material provides very effective valve seats that will eliminate sacrifices in strength and port configuration over conventional methods. In addition, because of better heat transfer, lighter weight valves can be utilized and larger valve areas can be employed so as to increase the performance of the engine without shortening its life. Of course, the foregoing description is that of the preferred embodiments of the invention, and various changes and modifications may be made without departing from the spirit and scope of the invention, as defined by the appended claims.

What is claimed is:

1. A cylinder head for an internal combustion engine comprised of a main cylinder head body formed from a first material comprising an aluminum alloy, said main cylinder head body being formed with a surface adapted to be in facing relationship to a cylinder block for closing a cylinder bore formed therein, a recess in said main cylinder head body surrounded by said surface, a flow passage extending through said cylinder head body between said recess and an external surface of said main cylinder head body, and a valve seat formed at the recess end of said flow passage by an insert formed from a Sintered ferrous alloy metallurgically bonded to the material of said cylinder head body at the

## 11

interface therewith by plastic deformation of said first material, said aluminum alloy having a solidus temperature greater than 530° C. to avoid significant melting thereof during the bonding process.

2. A cylinder head as set forth in claim 1, wherein the solidus temperature of the first material is about 555° C.

3. A cylinder head as set forth in claim 2, wherein the first material has a 0.2% yield strength at 400° C. less than 45 MPa.

4. A cylinder head as set forth in claim 3, wherein the first material has a 0.2% yield strength at 400° C. in the range of 30–35 MPa.

5. A cylinder head as set forth in claim 4, wherein the first material has a heat conductivity of greater than 120° C. W/m.

6. A cylinder head as set forth in claim 5, wherein the first material has a heat conductivity of about 160° C. W/m.

7. A cylinder head as set forth in claim 6, wherein the first material has an electrical resistivity of less than  $8.5 \times 10^{-2} \mu\Omega$ .

8. A cylinder head as set forth in claim 7, wherein the first material has an electrical resistivity of about  $7 \times 10^{-2} \mu\Omega$ .

9. A cylinder head as set forth in claim 8, wherein the alloying material of the first material is comprised of aluminum, silicon and magnesium.

10. A cylinder head as set forth in claim 2, wherein the first material has a heat conductivity of greater than 120° C. W/m.

11. A cylinder head as set forth in claim 10, wherein the first material has a heat conductivity of 160° C. W/m.

12. A cylinder head as set forth in claim 2, wherein the first material has an electrical resistivity of less than  $8.5 \times 10^{-2} \mu\Omega$ .

13. A cylinder head as set forth in claim 12, wherein the first material has an electrical resistivity of about  $7 \times 10^{-2} \mu\Omega$ .

14. A cylinder head as set forth in claim 2, wherein the alloying material of the first material is comprised of aluminum, silicon and magnesium.

15. A cylinder head for an internal combustion engine

comprised of a main cylinder head body formed from a first material, said main cylinder head body being formed with a surface adapted to be in facing relationship to a cylinder block for closing a cylinder bore formed therein, a recess in said main cylinder head body surrounded by said surface, a

flow passage extending through said cylinder head body between said recess and an external surface of said main cylinder head body, and a valve seat formed at the recess end of said flow passage by an insert formed from a second

material comprising a Sintered ferrous alloy metallurgically

## 12

bonded by plastic deformation to said main cylinder head body, said first material comprising an aluminum alloy having a 0.2% yield strength at 400° C. less than 45 Mpa for establishing plastic flow thereof during the bonding process to avoid significant melting thereof during the bonding process.

16. A cylinder head as set forth in claim 15, wherein the first material has a 0.2% yield strength at 400° C. in the range of 30–35 MPa.

17. A cylinder head for an internal combustion engine comprised of a main cylinder head body formed from a first material, said main cylinder head body being formed with a surface adapted to be in facing relationship to a cylinder block for closing a cylinder bore formed therein, a recess in

15 said main cylinder head body surrounded by said surface, a flow passage extending through said cylinder head body between said recess and an external surface of said main cylinder head body, and a valve seat formed at the recess end of said flow passage by an insert formed from a second

20 material comprising a Sintered ferrous alloy metallurgically bonded by elastic deformation to said main cylinder head body, said first material comprising an aluminum alloy having a 0.2% yield strength at 400° C. less than 45 Mpa for establishing plastic flow thereof during the bonding process

25 to avoid significant melting thereof during the bonding process.

18. A cylinder head as set forth in claim 17, wherein the first material has a heat conductivity of about 160° C. W/m.

19. A cylinder head for an internal combustion engine

30 comprised of a main cylinder head body formed from a first material, said main cylinder head body being formed with a surface adapted to be in facing relationship to a cylinder block for closing a cylinder bore formed therein, a recess in

35 said main cylinder head body surrounded by said surface, a flow passage extending through said cylinder head body between said recess and an external surface of said main cylinder head body, and a valve seat formed at the recess end of said flow passage by an insert formed from a Sintered

40 ferrous alloy metallurgically bonded by plastic deformation to said main cylinder head body by a process including electrical resistance heating, said first material comprising an aluminum alloy and having an electrical resistivity of less than  $8.5 \times 10^{-2} \mu\Omega$  for limiting the temperature attained during the bonding process to avoid significant melting

45 thereof during the bonding process.

20. A cylinder head as set forth in claim 19, wherein the first material has an electrical resistivity of about  $7 \times 10^{-2} \mu\Omega$ .

\* \* \* \* \*

UNITED STATES PATENT AND TRADEMARK OFFICE  
CERTIFICATE OF CORRECTION

PATENT NO. : 5,848,579  
DATED : December 15, 1998  
INVENTOR(S) : Adachi et al.

Page 1 of 1

It is certified that error appears in the above-identified patent and that said Letters Patent is hereby corrected as shown below:

Column 12, claim 17,  
Line 21, "elastic deformation" should be -- plastic deformation --.

Signed and Sealed this

Twenty-fifth Day of December, 2001

Attest:

Attesting Officer



JAMES E. ROGAN  
Director of the United States Patent and Trademark Office